

1

3,297,574  
LUBRICATING COMPOSITIONS CONTAINING  
EP AGENTS

Alexander C. B. MacPhail, Little Sutton, Francis T. Barcroft, Upton-by-Chester, and Charles B. Milne, Little Sutton, England, assignors to Shell Oil Company, New York, N.Y., a corporation of Delaware  
No Drawing. Filed Jan. 20, 1964, Ser. No. 338,588  
Claims priority, application Great Britain, Feb. 21, 1963,  
7,013/63

7 Claims. (Cl. 252—46.7)

This invention relates to synthetic lubricating compositions capable of functioning over a wide temperature range and under extreme pressure and wear conditions. More particularly the invention relates to synthetic ester base lubricating compositions which are stable and possess excellent extreme pressure and antiwear properties.

It is known that esters of mono or polyhydric alcohols and aliphatic dicarboxylic acids such as di(2-ethylhexyl)sebacate or esters of pentaerythritol and monocarboxylic acids such as C<sub>8</sub>—C<sub>18</sub> aliphatic carboxylic acids are acceptable base oils for aircraft gas turbine engines when inhibited with suitable antioxidants such as phenothiazine. However, lubricants of this type lack desired extreme pressure and antiwear properties and attempts to incorporate conventional extreme pressure agents such as organic phosphates or thiophosphates, sulfur-containing compounds and the like have met with little success.

It is an object of the present invention to provide improved high-temperature synthetic lubricating compositions. It is a further object of this invention to provide stable gas turbine engine synthetic lubricants with excellent extreme pressure and antiwear properties. Other objects will become apparent from the following description of the invention.

It has now been discovered that improved extreme-pressure properties are imparted to an aliphatic acid ester lubricating oil by the addition of minor amounts of each of (1) a chlorinated polyaryl compound and (2) a triaryl ester of phosphorothionic acid. More specifically, improved lubricating compositions of the invention comprise:

- (A) An aliphatic carboxylic ester lubricating base;
- (B) A minor amount of one or more chlorinated polyaryl hydrocarbons represented by the formula



where Ar is a mono or polynuclear aromatic hydrocarbon such as benzene, naphthalene, or anthracene, preferably at least one of which is benzene, x and y are integers of from 1 to 8 and preferably from 2 to 4, the chlorine atoms being attached directly to the carbon atoms of the aromatic nuclei, and z is an integer from 1 to 10, preferably from 1 to 4; and

- (C) A minor amount of a triaryl ester of phosphorothionic acid, each aryl group containing 6 to 10 carbon atoms.

2

The chlorinated polyaryl compounds described as additive (B) above are used in concentrations between about 0.5% and about 10% by weight and preferably between 1% and 6% by weight of the lubricating oil compositions. Compounds of this type include chlorinated and fluorinated diphenyl, triphenyl, tetraphenyl, pentaphenyl, phenylnaphthyl and mixtures thereof. The halogen content of these compounds varies from 20% to 80% by weight, preferably 40% to 70% by weight. A class of compounds of this type are commercially available under the trade name "Aroclor" from Monsanto Chemical Company. Particularly preferred are chlorinated (40—70%) diphenyls commercially available as "Aroclor 1254" and "Aroclor 1248," the former being a 40% chlorinated diphenyl. Although these compounds themselves produce desirable extreme pressure characteristics in synthetic lubricating oils, the desirable effects of these compounds do not substantially increase with a corresponding increase of additive concentration. In other words, although the addition of a small amount of these compounds imparts desirable properties to the oil, addition of increased amounts does not produce the expected further increase in extreme pressure properties. The low rate of increase of scuffing load with increasing Arochlor concentration is shown in Tables I and II, Examples II—IV below.

In accord with the present invention, the extreme pressure effect of the chlorinated polyaryl compounds is considerably enhanced by the addition of 0.5 to 10%, preferably 1 to 6% by weight of the lubricating oil composition, of a triaryl ester of phosphorothionic acid (additive (C) above). Addition of the prescribed amount of these esters surprisingly increases the effectiveness of the chlorinated polyaryl additive; i.e., as the concentration of chlorinated polyaryl is increased in the presence of a constant amount of triaryl phosphorothionate, there is a corresponding large increase in anti-scuff properties. Thus, the combination of these additives produces excellent extreme-pressure properties not attainable with the conventional chlorinated polyaryl additive alone. In Tables I and II, Examples VI—VIII below, it is shown that the rate of increase of scuffing load with increasing Arochlor concentration in the presence of 2% triphenyl phosphorothionate is considerably higher than in the absence of this compound. The resulting lubricating oil has excellent extreme-pressure properties which are only available with the use of the phosphorothionate additive.

Several compositions with varying Arochlor concentration, with and without triphenyl phosphorothionate, were tested for their load-carrying capacity on an I.A.E. Gear Rig as described in the Institute of Petroleum Method 166/60T using BSS-EN34 steel gears and operating at an oil temperature of 60° V. or 110° C. The mean failure loads at 2000 r.p.m. and 6000 r.p.m. were determined for the compositions of Table I and are shown in Table II.

TABLE I

| Composition of Example                          | I     | II   | III  | IV   | V    | VI   | VII  | VIII |
|-------------------------------------------------|-------|------|------|------|------|------|------|------|
| Di(isooctyl azelate), percent w.                | 100.0 | 94.0 | 95.0 | 92.0 | 95.0 | 92.0 | 93.0 | 90.0 |
| Aroclor 1254 (chlorinated diphenyl), percent w. |       | 3.0  | 5.0  | 8.0  |      | 2.0  | 3.0  | 5.0  |
| Triphenyl phosphorothionate, percent w.         |       |      |      |      |      | 1.5  | 1.5  | 2.0  |
| 3,7-Diethyl phenothiazine, percent w.           |       | 1.5  |      |      |      | 25   | 25   |      |
| 5-Methyl benzotriazole, p.p.m.                  |       | 25   |      |      |      |      | 5    |      |
| D.C. 200/12,000 silicone, p.p.m.                |       | 5    |      |      |      |      | 5    |      |
| Phenyl- $\alpha$ -naphthylamine, percent w.     |       | 1.5  |      |      |      | 1.5  | 1.5  |      |

TABLE II

| Example                                                                    | I   | II  | III | IV  | V   | VI  | VII | VIII |
|----------------------------------------------------------------------------|-----|-----|-----|-----|-----|-----|-----|------|
| I.A.E. Scuffing Load, lbs.:<br>2,000 r.p.m.—                               |     |     |     |     |     |     |     |      |
| 60° C.—                                                                    | 45  | 55  | 70  | 75  | 90  | 100 | 110 | >120 |
| 110° C.—                                                                   | 45  | 74  | 70  | 75  | 80  | 105 | 110 | >120 |
| 6,000 r.p.m.—                                                              |     |     |     |     |     |     |     |      |
| 60° C.—                                                                    | 35  | 45  | 47  | 50  | 40  | 40  | 65  | 85   |
| 110° C.—                                                                   | 25  | 34  | 37  | 40  | 45  | 30  | 60  | 85   |
| Sum of scuffing loads, lbs.                                                | 150 | 208 | 224 | 240 | 255 | 275 | 345 | >410 |
| Increase of scuffing loads with increasing Aroclor concentration           |     |     |     |     |     |     |     |      |
| Rate of increase of scuffing load per 1% increase in Aroclor concentration | 58  | 16  | 16  |     |     | 20  | 70  | >65  |
|                                                                            | 19  | 8   | 5   |     |     | 7   | 35  | >22  |

Examples of triaryl esters of phosphorothionic acid suitable for use in compositions of the invention are triphenyl phosphorothionate, tritolyl phosphorthinate, tribenzyl phosphorothionate, and trixylyl phosphorothionate. The preferred ester is triphenyl phosphorothionate.

The aliphatic carboxylic acid ester lubricating oil bases which are used in lubricating oil compositions according to the invention may be esters of a monohydric aliphatic alcohol having from 3 to 18 carbon atoms in the molecule, with a monobasic aliphatic acid having from 4 to 18 carbon atoms in the molecule, for example isodecyl pelargonate.

A further class of aliphatic carboxylic acid esters which may be used is the aliphatic esters of monobasic carboxylic acids having from 4 to 18 carbon atoms and a glycol having from 4 to 20 carbon atoms, for example esters of neopentyl glycol, 2-butyl-2-ethyl-1,3-propanediol and dipropylene glycol, with heptylic acid, n-octoic acid and pelargonic acid.

A particularly preferred class of aliphatic acid esters for use in the lubricating oil compositions of the invention is the aliphatic diester of diabasic carboxylic acids having 6 to 20 carbon atoms and monohydric alcohols having from 1 to 12 carbon atoms, for example esters of adipic acid, pimelic acid, suberic acid, azelaic acid and sebatic acid with lauryl alcohol, heptyl alcohol, octyl alcohol and nonyl alcohol. Particularly preferred aliphatic diesters of dicarboxylic acids are those derived from monohydric alcohols having a branched chain, for example 2-ethyl hexanol and especially those having no hydrogen on the beta carbon atom, for example 2,2-dimethyl pentanol, 2,2,4-trimethyl pentanol, 2,2,3-trimethyl pentanol, 2,2-dimethylhexanol, and 2-methyl-2-ethyl hexanol.

As examples of other aliphatic carboxylic acid esters which may be used there are mentioned aliphatic esters of monocarboxylic acids having from 3 to 10 carbon atoms, for example, propionic acid, butyric acid, valeric acid, capric acid, caprylic acid, lauric acid and pelargonic acid and polyols, for example, pentaerythritol, dipentaterythritol and trimethylolpropane.

Examples of such esters are pentaerythrityl butyrate, pentaerythrityl tetrabutyrate, pentaerythrityl tetravalerate, pentaerythrityl tetracaproate, pentaerythrityl dibutyratadicaprate, pentaerythrityl butyratecaproate divalerate, pentaerythrityl butyrate trivalerate, pentaerythrityl butyrate tricaproate, pentaerythrityl tributyratcaproate, mixed  $C_{4-6}$  saturated fatty acid esters of pentaerythritol, dipentaerythrityl hexavalerate, dipentaerythrityl hexacaproate, dipentaerythrityl hexaheptoate, dipentaerythrityl hexacaprylate, dipentaerythrityl tributyratcaproate, dipentaterythrityl trivalerate trinonylate, dipentaerythrityl mixed hexaesters of  $C_{4-10}$  fatty acids and trimethylolpropane heptylate.

A class of pentaerythritol esters useful as base oils are Hercules "Hercoflex" and "Hercolube" pentaerythritol esters such as "Hercoflex 600 and 900," "Hercolube J69" which are dipentaerythritol esters of an alkanoic acid selected from the group consisting of alkanoic acids having from 5 to 10 carbon atoms and mixtures of alkanoic acids having from 2 to 12 carbon atoms in proportions to provide an average chain length of from 5 to 10 carbon

15 atoms. "Hercolube A" and "Hercolube C" ( $C_8-C_{10}$  and  $C_4-C_6$  acid esters of pentaerythritol) and "Hercolube F" ( $C_8-C_{10}$  acid esters of dipentaerythritol) are particularly useful base oils for the additives of the invention.

The aliphatic carboxylic acid esters need not necessarily be simple esters or mixtures thereof but may be what are termed "complex esters" made by esterifying in one or more stages, an aliphatic dicarboxylic acid and a glycol or polyglycol optionally together with an aliphatic monocarboxylic acid and/or an aliphatic monohydric alcohol. A typical complex ester is that made by esterifying two moles of an aliphatic dicarboxylic acid, one mole of a glycol or polyglycol and two moles of an aliphatic monohydric alcohol having a formula:



30 wherein  $R$  is an alkylene or oxyalkylene group,  $R_1$  is an alkylene group, and  $R_2$  is an alkyl group.

Preferred complex esters of the type are those wherein  $R$  is an alkylene or oxyalkylene group having from 2 to 20 carbon atoms,  $R_1$  is an alkylene group, optionally branched chained, having from 6 to 20 carbon atoms, and  $R_2$  is an alkyl group, preferably branched chained and especially having no hydrogen atoms on the beta carbon atom, having from 1 to 12 carbon atoms.

40 Mixtures of the above-described aliphatic carboxylic acid esters may also be used in the lubricating oil compositions according to the invention. Especially suitable mixtures are those of the aliphatic esters of dicarboxylic acids and branched chained monohydric alcohols and the complex esters as defined above. The "complex esters" have the effect of thickening the lubricating oil composition which is especially valuable when the lubricating oil is required for the lubrication of British aircraft turbine engines operating on a lubricant having a viscosity of 7.5 cs. at 210° F.

50 The lubricating oil compositions of the invention may contain any of the known additives for aliphatic carboxylic acid ester lubricating oils, for example thickeners, anti-oxidants, antilacquering agents, anti-foaming agents, dyes, anti-corrosion agents, metal deactivators and additional extreme pressure additives if necessary.

As thickeners there may be used polyalkylene glycols and their mono- and di-ethers or -esters having the general formula



wherein  $R_1$  and  $R_3$  each represent a hydrogen atom, a non-aromatic hydrocarbon radical or an acyl group,  $R_2$  represents an alkylene radical and  $n$  represents an integer. In the polyoxyalkylene chain  $-(R_2O)_n-$ , the radical  $R_2$  may be an alkylene radical, preferably an alkylene radical with two to eight carbon atoms. Still more preferred polyalkylene glycols are those wherein the alkylene radical is an ethylene or propylene radical. In the polyoxyalkylene chain  $-(R_2O)_n-$  there may be present alkylene radicals with different numbers of carbon atoms.

70 The chain may, for instance, consist of both oxyethylene and oxypropylene radicals. In the instance where the polyoxyalkylene chain contains different alkylene radicals, these may be randomly distributed throughout the molecule or may be arranged in regularly recurring units or

blocks, each consisting of one or a plurality of similar oxyalkylene radicals. Particularly preferred polyalkylene glycols are those having blocks of, for example, 1 to 8 oxyethylene radicals alternating with blocks of, for example, 1 to 8 oxypropylene radicals.

In those cases where the radicals represented in the above general formula by  $R_1$  and/or  $R_2$  are hydrocarbon radicals, the radicals may be saturated or unsaturated, straight chained or branched, or similar or dissimilar, non-aromatic hydrocarbon radicals. A particular preference is given to polyalkylene glycols in which  $R_1$  is hydrogen and  $R_3$  is an alkyl group such as a propyl, butyl, pentyl or decyl group.

In those cases where the radicals  $R_1$  and/or  $R_3$  are acyl radicals, the radicals may be derived from any carboxylic acid. Preference is given to the alkane or alkene monocarboxylic acids such as acetic acid, propionic acid, butyric acid, lauric acid, stearic acid and oleic acid.

The molecular weight of the polyalkylene glycols may vary over a wide range but preferably is from 350 to about 10,000; molecular weights between 800 and 6,000 are particularly preferred. The polyalkylene glycol thickener may be used in a concentration of between 5% and 50%, preferably between 15% and 40% based on the whole composition.

Suitable polyalkylene glycols are those sold under the name Ucon Fluids (the word "Ucon" is a Registered Trademark) manufactured by the Carbide and Chemical Corporation and Oxilube (the word "Oxilube" is a trademark) manufactured by Shell Internationale Chemical Company and are described in U.S. Patents 2,425,755, 2,425,845 and 2,952,335. "Ucon" fluids of the LB-X series made by copolymerizing ethylene oxide and 1,2-propylene oxide and having viscosities (at 100° F.) of about 140 and 370 cs. respectively have been found to give excellent results.

As antioxidants which may be used in the lubricating oil composition according to the invention there are mentioned alkylated phenols, for example 2,6-ditertiary butyl-4-methyl phenol, alkylated bisphenols, for example 4,4'-methylene bis(2,6-ditertiary butyl phenol), aromatic amines, for example phenyl- $\alpha$ -naphthylamine, phenyl- $\beta$ -naphthylamine, diphenylamine and alkyl substituted derivatives thereof.

An especially preferred class of antioxidants is the thiadialyamines, for example phenothiazine and 3,6-diethylphenothiazine. Mixtures of antioxidants may also be used, particularly mixtures of thiadialyamines and diaryl-aminies, for example a mixture of phenothiazine and phenyl- $\alpha$ -naphthylamine.

Other optional additives for the present lubricating oil compositions are anti-foaming agents, for example polydimethylsiloxanes having viscosities from 100-100,000 cs. at 25° C., anti-corrosion agents, and metal deactivators, for example benzotriazole and 5-methylbenzotriazole.

We claim our invention:

1. A synthetic lubricating oil comprising

(1) a major amount of an aliphatic carboxylic acid ester oil base,

(2) about 0.5% to about 10% by weight of a chlorinated polyaryl hydrocarbon having the formula



where Ar is selected from the group consisting of mono- and polynuclear aromatics,  $x$  and  $y$  are integers of from 1 to 8, and  $z$  is an integer of from 1 to 10, and

(3) about 0.5% to about 10% by weight of a triaryl ester of phosphorothionic acid, each aryl group having 6 to 10 carbon atoms.

2. The synthetic lubricating oil composition of claim 1 wherein the triaryl ester of phosphorothionic acid is triphenyl phosphorothionate.

3. The composition of claim 1 wherein the aliphatic carboxylic acid ester oil base consists essentially of an aliphatic diester of dibasic carboxylic acids having from 6 to 20 carbon atoms and monohydric alcohols having from 1 to 12 carbon atoms.

4. A synthetic lubricating oil composition comprising

(1) a major amount of an aliphatic carboxylic acid ester oil base,

(2) about 0.5 to about 10% by weight of a chlorinated polyaryl hydrocarbon having the formula



wherein Ar is an aromatic hydrocarbon selected from the group consisting of benzene, naphthalene, and anthracene,  $x$  and  $y$  are integers of from 1 to 8, and  $z$  is an integer of from 1 to 10, and

(3) about 1% to 6% by weight of a triaryl ester of phosphorothionic acid, each aryl group having 6 to 10 carbon atoms.

5. The composition of claim 4 wherein the triaryl ester of phosphorothionic acid is triphenyl phosphorothionate.

6. The composition of claim 4 containing an antioxidant selected from the group consisting of 2,6-ditertiary butyl-4-methyl phenol; 4,4'-methylene bis(2,6-ditertiary butyl phenol), phenyl  $\alpha$ -naphthylamine, phenyl  $\beta$ -naphthylamine, diphenylamine, phenothiazine, and 3,6-diethylphenothiazine.

7. A synthetic lubricating oil comprising a major amount of an aliphatic carboxylic acid ester oil base, 0.5 to 10% by weight of diphenyls containing 40 to 70% by weight chlorine, and 1 to 6% by weight of triphenyl phosphorothionate.

50 References Cited by the Examiner

UNITED STATES PATENTS

|           |         |                |       |          |
|-----------|---------|----------------|-------|----------|
| 2,157,452 | 5/1939  | Humphreys      | ----- | 252—46.6 |
| 2,242,260 | 5/1941  | Prutton        | ----- | 252—46.7 |
| 2,820,766 | 1/1958  | Elliott et al. | ----- | 252—46.6 |
| 3,030,304 | 4/1962  | Elliott et al. | ----- | 252—46.7 |
| 3,218,256 | 11/1965 | Edwards et al. | ----- | 252—47.5 |

55 DANIEL E. WYMAN, Primary Examiner,

60 L. G. XIARHOS, Assistant Examiner,